

## UNITED STATES PATENT OFFICE

TADASHI TANABE, OF TORIGAI, FUKUOKA, JAPAN

## STAINLESS SILVER ALLOY

No Drawing. Application filed February 12, 1932, Serial No. 592,861, and in Japan February 17, 1931.

The present invention relates to stainless silver alloy which contains 0.5 to 20.0% of zinc, 10.0 to 40.0% of tin and 50.0 to 89.5% of silver, and the object thereof is to obtain such silver alloy as is hardly stained by air or moisture, especially by sulphides and is easy to cast and work.

In order to manufacture the silver alloy according to this invention, firstly red-heat 10 a crucible in a suitable furnace and charge it with pure silver for melting, preventing the oxidation of the metal by adding flux such as borax to cover the said metal. After adding the desired quantity of tin and zinc thereto and melting them, together, stir the mixture and then leave it alone for several minutes. When it has settled, pour it into a mold.

Now, with regard to a binary alloy 20 consisting of tin or zinc added separately to silver, the quantity of the material to be added must be pretty large to maintain the alloy in a stainless condition. However, an alloy which contains a large quantity of such material does not only lose the peculiar silvery lustre, but is too hard and brittle to be worked, whereas the alloy according to this invention which is manufactured by adding tin and zinc at the same time is quite 25 free from such defect. It does not only have the lustre peculiar to silver alloy, but is almost stainless. Moreover, it is tough enough for working.

In the alloy manufactured by adding tin 30 and zinc simultaneously to silver, if the quantity to be added is small, the alloy maintains silver color and is so soft that it is easy to work, but if the quantity is too large, it more or less loses silver color, increasing both 35 hardness and brittleness and consequently being difficult to work. Therefore, as the results of experiments the following restriction has been put to the quantity of tin and zinc to be added.

40 The following experiment shows clearly

that according to the present invention the hardness of the alloy increases with the quantity of zinc. By the way, in this experiment the percentage of the weight of tin content is kept at 30% and the quantity of zinc content 50 is increased gradually.

| Test pieces | Ingredients and per cent of their weight |      |        | Hardness | 55 |
|-------------|------------------------------------------|------|--------|----------|----|
|             | Zinc                                     | Tin  | Silver |          |    |
| A           |                                          |      |        | 100.0    | 23 |
| B           | 0.5                                      | 30.0 | 69.5   | 42       |    |
| C           | 5.0                                      | 30.0 | 65.0   | 59       |    |
| D           | 10.0                                     | 30.0 | 60.0   | 62       |    |
| E           | 15.0                                     | 30.0 | 55.0   | 85       | 60 |

*Remarks.*—The figures described in the "Hardness" column of the above table show Brinell's hardness numbers obtained in applying the load of 5 kilograms to the ball of 1 millimeter diameter for one minute.

The characteristic feature of the alloy of 65 this invention is that it is almost stainless and non-corrosive. For instance, ornamental articles, made of this alloy do not have their elegant appearance spoiled for a long time.

The following are the results of experiments made with the pieces mentioned before:—

(A) When the test pieces were polished uniformly with emery paper and immersed in decinormal solution of sodium sulphide 75 and their colored condition was compared with electrolytic silver (purity 99.98%) as the standard,

|                         |                                      |    |
|-------------------------|--------------------------------------|----|
| A (electrolytic silver) | Turned black entirely in ten minutes | 80 |
| B                       | Hardly colored                       |    |
| C                       | do                                   |    |
| D                       | do                                   |    |
| E                       | do                                   | 85 |

(B) When the test pieces were arranged on a glass dish and exposed in the open air for 6 months and their stainless was compared,

- A (electrolytic silver)—Turned black entirely in six months  
 B—Hardly discolored even after the lapse of six months  
 C—do  
 D—do  
 E—do

(C) The following color standards were made previously by polishing pure silver (purity 99.98%) uniformly with emery paper and immersing the same in decinormal solution of sodium sulphide for different time:—

| 15 | Standard color | Duration of immersion | Coloring                        |
|----|----------------|-----------------------|---------------------------------|
|    | No. 1          | 2 seconds             | Light yellow.                   |
|    | No. 2          | 5 seconds             | Brownish light yellow.          |
|    | No. 3          | 10 seconds            | Brownish red increased.         |
| 20 | No. 4          | 15 seconds            | Do.                             |
|    | No. 5          | 20 seconds            | Partially blue.                 |
|    | No. 6          | 30 seconds            | Bluish green increased.         |
|    | No. 7          | 40 seconds            | Brownish blue increased.        |
|    | No. 8          | 50 seconds            | Do.                             |
|    | No. 9          | 60 seconds            | Deep blue, but brown partially. |
|    | No. 10         | 2 minutes             | Brown disappeared.              |
|    | No. 11         | 5 minutes             | Almost grey.                    |
| 25 | No. 12         | 10 minutes            | Bluish dark grey.               |
|    | No. 13         | 20 minutes            | Do.                             |

When the test alloys according to this invention which consist of the following ingredients were polished uniformly with emery paper and their colors were compared with the above color standards after immersing them in decinormal sodium sulphide solution for ten minutes.

| 40 | Test pieces | Tin      | Zinc     | Silver     |
|----|-------------|----------|----------|------------|
|    |             | Per cent | Per cent |            |
|    | F           | 19.42    | 15.07    | Remainder. |
|    | G           | 23.12    | 8.11     | Remainder. |
|    | H           | 20.09    | 4.64     | Remainder. |
|    | K           | 18.43    | 11.72    | Remainder. |

  

| 45 | Test pieces | Coloring                                                                                                                                    |
|----|-------------|---------------------------------------------------------------------------------------------------------------------------------------------|
|    | F           | Below No. 1 of the color standards of pure silver. Nearly the same color as when pure silver is immersed in the above reagent for a second. |
|    | G           | Same as No. 2.                                                                                                                              |
|    | H           | Same as No. 1.                                                                                                                              |
|    | K           | Same as No. 1.                                                                                                                              |

Next, upon comparing the corosions due to chemicals of metallic silver, copper, zinc, tin and the alloy of this invention (tin 20% and zinc 10%),

(a) Corrosion test with salt solution. The above five kinds of test pieces were put separately in vessels and boiled for ten minutes with the addition of the same quantity of 5% common salt water, and then after left alone for 26 hours, they were taken out at the same time. After cleaning their surfaces with tooth brush, they were dried and weighed. When the change of their weight (gram)

was divided by the surface area (square centimeter) of the test pieces, the following figures were obtained:—

|                                   | Gr. sq. cm. |            |
|-----------------------------------|-------------|------------|
| Copper                            | Decrease    | 0.00070 70 |
| Zinc                              | Decrease    | 0.00043    |
| Tin                               | Decrease    | 0.00041    |
| Silver                            | Increase    | 0.00214    |
| Alloy according to this invention | Decrease    | 0.00016 75 |

*Remark.*—The increase of weight in silver is due to the film of silver chloride produced upon the surface of the test material.

(b) Corrosion test with acetic acid. After boiling the above five kinds of test pieces in 10% acetic acid solution for ten minutes by the same process with the above, they were left alone for 8 hours and the decrease of their weight was examined.

|                                   | Gr. sq. cm. |            |
|-----------------------------------|-------------|------------|
| Copper                            | Decrease    | 0.00038 85 |
| Zinc                              | Decrease    | 0.03889    |
| Tin                               | Decrease    | 0.00070    |
| Silver                            | Decrease    | 0.00050    |
| Alloy according to this invention | Decrease    | 0.00010 90 |

From the above tables it will be seen that in both of the tests (a) and (b) the alloy made according to this invention show the least decrease.

As already stated, the alloy of this invention is not only hardly colored but almost non-corrosive. As compared with the annealed pure silver which has the tensile strength of 14 kilograms per square millimeter, the elongation of 40% and the hardness (Brinell) of 23, it has the tensile strength of about 20 kilograms per square millimeter, the elongation of about 11% and the hardness (Brinell) of about 60. Thus, although it shows more or less decrease in the elongation as compared with pure silver, an increase is seen in the tensile strength and hardness. Consequently, it is so hard as to be suitable for the material for table-wares and other kinds of wares. Although there is more or less the decrease in its elongation, and the increase in the tensile strength and hardness, it is not so brittle as to be difficult to work. Now, pure silver in a fused state absorbs oxygen of the volume nearly twenty-three times as large and liberates it on solidification and is apt to produce gas holes in a cast article, whereas the alloy according to this invention containing zinc and tin which act as deoxidizers, they drive away the oxygen which would be absorbed in fused silver, thus making it possible to produce easily a cast article free from gas holes.

In short, this invention is characterized by the fact that the desired object can be accomplished quite satisfactorily in spite of few kinds of metals contained therein and the simpleness of the method of manufacture.

Therefore, it is most suitable as the material for table-wares, ornamental articles, watch cases, etc.

I claim.

5 A stainless alloy consisting of 0.5-20.0% of zinc, 10.0-40.0% of tin and 50.0-89.5% of silver.

TADASHI TANABE.

10

15

20

25

30

35

40

45

50

55

60

65